

# UNITED STATES PATENT OFFICE.

SAMUEL S. EDDY, OF ROCHESTER, NEW YORK.

## TANNING PROCESS.

SPECIFICATION forming part of Letters Patent No. 300,352, dated June 17, 1884.

Application filed April 10, 1884. (Specimens.)

*To all whom it may concern:*

Be it known that I, SAMUEL S. EDDY, a citizen of the United States, residing at Rochester, New York, have invented new and useful Improvements in Processes for Tanning, of which the following is a specification.

My invention relates to an improvement in the process of tanning, more especially to the tanning of those skins which it is desired to convert into kid-leather. Hitherto in tanning such skins it has been necessary, when taken from the pickle, (or what are known as pickled sheep-skins,) to extract or kill the pickle, and it has been found that the processes used therefor are apt to injure the skin and detract from the quality of the finished leather.

The object of my invention is to furnish a process by the use of which the tanning may proceed without killing or extracting the pickle which may be in the skin, and to produce economically a high grade of leather, always soft and pliable, and capable of receiving and reliably retaining and holding the color or dye imparted to it. The process by which this is effected is as follows: Suppose the number to be treated is twelve dozen sheep-skins taken from the pickle, (what are known as pickled sheep-skins.) For this number I make a first solution or composition of eighty-four pounds of wheat-bran fermented in one hundred and twenty gallons of water, seventy-five pounds of salt, fifteen pounds of sulphuric acid or oil of vitriol of 66° strength, and five pounds of quercitron bark. The bark should be boiled in four or five gallons of water, to extract the strength therefrom before mixing it with the other ingredients.

The composition thus made is intended for white leather. When it is intended to color the leather, it is preferable to add to the composition noted about eight pounds of terra-japonica dissolved in a suitable amount of water.

The ingredients of this solution possess qualities peculiarly adapting it for the desired effects on the skins. The wheat-bran tends to soften the skins, while at the same time it possesses mild tanning properties. The salt is cleansing in its action, as is also the oil of vitriol, while the two, when mixed, form a tan-

ning agent. The quercitron is a well-known tanning agent, giving body or strength to the composition and strengthening or toughening the skins.

55  
Into this composition the skins are thrown, preferably single, in order that every part of the skin may be affected thereby. They are to be kept therein about ten hours, when they should be taken out and washed off with or in luke-warm or cool water, and then hung upon a horse or rack and allowed to drain for an hour or more, when they are ready for a second solution or composition. This is composed of sixty gallons of water, three pints of 60 soft soap, one pound of glycerine, twelve ounces of saleratus, and six ounces of borax. The saleratus and borax should be separately dissolved in a little water before being added to the other ingredients.

70  
In this composition the use of the soap softens, cleanses, and strengthens the skins, while the glycerine, in addition to its preservative qualities, tends to keep them soft and pliable. The borax whitens and bleaches the skins, 75 while it and the saleratus, being alkalies, neutralize any acid remaining in the skins from their treatment in the first solution. In treating the skins in this solution it is preferable to treat a much smaller number at once than 80 the twelve dozen for which the entire solution is intended. It is best, therefore, to place about five gallons of this second composition in any suitable tub or receptacle, and place one dozen skins therein, which are then to be 85 handled in the solution for five minutes. This liquor is then to be thrown away and a fresh five gallons used with the next dozen in the same way, and so on until all the skins have had a five-minutes' handling in this second 90 composition. They are then to be hung up in a hot room until dry. After drying, they are to be seasoned by dipping quickly in water and packing in a box. They should remain so packed for some hours—ten or twelve, 95 or, say, over night—after which the next step is to perch out with the armstake, when they will be ready for the cleansing, which may be done in a solution composed of thirty-six gallons of water, six pounds of alum, and three 100 pounds of salt, in which they should be thoroughly handled for about five minutes. The

skins are now ready for dyeing or coloring and finishing, or for finishing, if white leather is desired. If to be colored, they are colored and worked in the manner usual with kid-  
5 finished leather. After a charge of the first solution or composition has been made of the strength and proportions set forth, and used as described, it may serve as a base for the next lot, as it may be strengthened and re-  
10 stored to its original activity by adding to what is left of it fifty pounds of bran fer-  
mented as before set out, five to six pounds of sulphuric acid, and twenty-five to thirty  
15 pounds of salt, with the necessary quantity of water. The second solution or composition, however, cannot be strengthened and must be made fresh for each lot to be treated, the spent liquor being simply thrown away.

While I have stated what I conceive to be  
20 the best proportions of ingredients for the solutions or compositions used, it is of course evident that they may be somewhat varied to meet the conditions of different qualities of skins.

25 It will be noted that the conjoint action of both compositions one and two, though used at different times, is needed to complete the tanning, the preliminary step being accom-  
plished by the first composition, which is an  
30 acid tanning solution, when action is supple-  
mented and finished by the second, which is an alkaline tanning solution, their action be-  
ing aided by the intervening and succeeding  
35 operations of washing, draining, and packing,  
the final solution acting as an ordinary cleans-  
ing solution after the changes necessary to

40 forming leather have been completed in the hide, the pickle in the hides having been neu-  
tralized by the conjoint effect of the acid and the alkaline tanning solutions.

With these compositions and by this method  
of treatment I am enabled to proceed with  
the tanning of pickled skins without first kill-  
ing or extracting the pickle, and to easily and  
economically produce a strong leather of the 45  
highest and best kid finish, soft and pliable,  
and capable of receiving a good color and  
durably retaining and holding it. The leather  
produced is also free from any bad or offend-  
50 ing odor, the effect of the compositions used  
being to destroy any such odors which might  
arise from the decomposition or change in the  
animal fibers.

Having thus described my invention, what  
I claim is—

55 The improved method of tanning pickled  
hides, or hides fresh from the pickle, which  
consists in first partially tanning by subject-  
ing them in the pickled condition to an acid-  
ulating composition substantially of the char-  
acter set forth, then washing and draining,  
60 and next completing the operation of tanning  
by the action of an alkaline tanning composi-  
tion substantially of the character set forth,  
and then drying.

65 In testimony whereof I affix my signature in  
presence of two witnesses.

SAMUEL S. EDDY.

Witnesses:

H. H. PYOTT,  
F. M. EDDY.